

## UNITED STATES PATENT OFFICE

2,538,279

MANUFACTURE OF ARTICLES COMPRISING  
CELLULOSE

Wayne A. Sisson, Silverside, and Mamerto M. Cruz, Jr., Wilmington, Del., assignors to American Viscose Corporation, Wilmington, Del., a corporation of Delaware

No Drawing. Application November 30, 1944,  
Serial No. 566,016

12 Claims. (Cl. 18—54)

1

This invention relates to methods of handling acid-moist articles comprising partially regenerated cellulose whereby to protect the same from deterioration due to acid-degradation of the cellulose, upon completion of regeneration of the cellulose.

Articles formed from viscose by extruding or casting the viscose into an acid setting bath always carry an appreciable quantity of adhering acid from the bath. For reasons of economy, the viscose is extruded or cast into the acid bath continuously, and the articles thus formed are passed through the bath and withdrawn therefrom rapidly, so that the viscose is only partially coagulated or "set up" when the article emerges from the bath. Articles so obtained comprise a skin of cellulose hydrate enveloping fluid viscose or only partially decomposed xanthate, dependence being placed upon penetration of the adhering acid through the skin to complete the decomposition of the cellulose xanthate. While the chemical reactions leading to such xanthate decomposition are in progress, the presence of the acid is necessary, and the acid does not exert an appreciable over-all degrading effect on the cellulose which has been regenerated. However, after all of the cellulose xanthate has been decomposed, the free sulphuric acid attacks the cellulose, with the result that the quality of the article is effected. For instance, in the case of filamentary material, if free acid is permitted to remain on the material for any appreciable time after the cellulose is regenerated, acid degradation or "tendering" of the cellulose is soon evidenced by a lowering of the D. P. number (Degree of Polymerization) indicating a change in the molecular structure, and resulting in diminished tensile strength and extensibility of the filaments.

For this reason, it is the common practice to subject acid-moist articles comprising regenerated cellulose to washing with water as soon as practicable after withdrawal of the article from the acid bath and completion of regeneration of the cellulose, in order to remove the acid therefrom.

However, it frequently happens that there is a considerable time lapse between withdrawal of the articles from the acid bath, and washing thereof, during which time any cellulose xanthate present is completely decomposed, and the regenerated cellulose is subject to acid attack. Such delays may be occasioned by a temporary breakdown of the washing equipment, by the necessity for storing the acid-moist articles during

2

overnight or longer plant shutdowns, or for other reasons. The occasional occurrence of such unavoidably long intervals between completion of regeneration of the cellulose and removal of the acid from the articles has been a source of difficulty in the rayon industry because even a slight percentage of cellulose degradation has a pronounced effect on the life of articles made therefrom.

10 It is a general object of the present invention to provide a method of handling acid-moist articles comprising partially regenerated cellulose so that the acid is prevented from exerting a degrading action on the cellulose. It is another object of the invention to prolong the period during which acid-moist articles comprising partially regenerated cellulose may be stored safely, prior to washing thereof, without inhibiting decomposition of any cellulose xanthate present.

15 The instant invention is based upon our discovery that the rate at which dethanthylation of cellulose xanthate proceeds to completion in the presence of acid, and the onset of acid degradation of the regenerated cellulose are functions 20 of the pH on the article, both dethanthylation and acid degradation being accelerated at extremely low pH, especially at higher temperatures such as may prevail in storage cabinets or the like, and depending to some extent on the length of time during which the article is permitted to stand in the acid moist condition.

25 The acid-laden articles as they come from the setting bath normally have a pH below about 0.5. As such low pH, the onset of acid-degradation of the cellulose is noticeable even after only short periods of standing.

We have now discovered that when it is necessary for any reason to store acid-moist articles comprising partially regenerated cellulose for any appreciable length of time, an equilibrium can be established between the rate at which dethanthylation is completed and the rate at which acid-degradation is effected, by controlling the pH on the article so that it is raised to and maintained at a value greater than 1 and less than 7. It is preferred to maintain the pH on the article at from 2 to about 3.5, and specifically at about 2.5, because at such a pH value acid-degradation is substantially entirely eliminated, irrespective of other existing conditions, such as temperature, the length of time during which the article is stored, and the concentration of the acid on the article, while at a pH lower than 2 acid-degradation may be quite noticeable at the 50 higher temperatures, say temperatures of 100° C.

or higher. Illustratively, and preferably, this objective may be accomplished by permitting the article to stand in the presence of an aqueous solution of sodium sulfate. Instead of an aqueous solution of sodium sulfate, solutions of other sodium salts may be substituted including sodium phosphate, acetate, phthalate, etc. Again, buffering systems may be used. The concentration of the aqueous sodium salt solution may vary somewhat depending upon the particular salt employed but in general solutions of 10 to 30% concentration are serviceable. For example, when aqueous solutions of sodium sulfate are employed, solutions of 15 to 20% concentration are preferred.

We found, for example, that when wound packages (weight approximately 3.5 lbs.) of freshly spun acid-moist yarn produced from viscose in accordance with the wet spinning process, and having a pH of below 0.5 were immersed in six liters of a 16% aqueous solution of sodium sulfate having a pH of 6.1, at room temperature, a pH of about 3.1 was established after about one hour. The pH gradually dropped to about 2.5. After standing in the solution for about 530 hours, the yarn after washing with water and drying at room temperature, was found to have a D. P. number (Degree of Polymerization) as measured by the cuprammonium viscosity method (Battista Ind. & Eng. Chem. Analytical Ed. vol. 16, pg. 351, June 1944) of 399, as contrasted with the D. P. number of the material before immersion, which was 412, i. e., after standing for 530 hours the drop in D. P. number was only 3.9%, and the yarn had a dry tensile strength of 2.66 gms./denier and dry extensibility of 18.4%; wet tensile strength of 1.66 gms./denier and wet extensibility of 27.5%. On the other hand, when similar wound packages of acid-moist yarn, produced in the same manner, and having a pH of below 0.5 were stored in a cabinet at room temperature and exposed to circulating air at relative humidity of 90%, for 530 hours, the yarn had a D. P. number of 221, that is, the drop in D. P. of the yarn at the end of that period was 46.3%, and the yarn had a dry tenacity of only 1.8 gms./denier, dry extensibility of 10.8%, wet tenacity of 0.84 gms./denier and wet extensibility of 9.4%.

If the pH on the article is adjusted to and maintained at a value of greater than 1 and less than 7 in accordance with this invention, partially regenerated cellulose articles which carry adhering acid may be stored safely for prolonged periods, even though the pH is on the acid side. This is indeed surprising in view of the general knowledge as to the deterioration of cellulose at acid pH's and the recognition of the art as to the ill-effects incident to departing from the standard practice of washing cellulose articles obtained from viscose by the wet spinning method within a short period of time after formation thereof.

In addition to preventing or markedly inhibiting acid degradation of cellulosic articles during storage, the invention has ancillary advantages. Thus, when wound packages of filamentary material are treated the yarn does not dry out and crystallization of salts, such as may have been carried from the spinning bath and which cause breaking of the yarn, does not occur within the package, with the result that the yarn finally obtained is of good quality and characterized by uniform strength and shrinkage and dyeing capacities along the entire length thereof. The in-

vention is of special value when acid-moist filamentary material derived from viscose and destined for use in the manufacture of tires is stored, because even a very small percentage of acid-degradation has a markedly pronounced deleterious effect on the flexing life of tire cord.

The acid-moist article comprising cellulose may be steeped or immersed in the aqueous sodium salt solution, or the latter may be sprayed or otherwise applied to the article after withdrawal thereof from the setting bath. For example, the solution may be sprayed or poured on filamentary material as it is withdrawn from the spinning bath, in which case the solution remains on the material after collection thereof. The aqueous sodium salt solution may serve as a plasticizing agent during stretching of the filaments and may be applied to the material as it advances over the stretching reel or other stretching device of a continuous spinning system. The solution may also be applied to filamentary material produced by a continuous spinning method, to complete dextranization of the cellulose xanthate prior to subjecting the material to the usual after-treatments. When the solution is applied as a plasticizer during stretching or to complete dextranization or when applied for both purposes in succession, it is preferably heated to a temperature of from about 60° C. to just below 100° C.

Certain variations and modifications may be made in practicing the invention without departing therefrom and it is to be understood that we are not to be limited except by the spirit and scope of the appended claims.

We claim:

1. The method of handling acid-moist articles freshly prepared from viscose, which articles comprise at least some partially regenerated cellulose and have a pH of less than 1 after withdrawal thereof from an acid setting bath, to effect complete regeneration of the cellulose by the acid while inhibiting acid degradation of the cellulose during and after such regeneration, and while the articles are held under acidic conditions comprising storing the article, at room temperature and under atmospheric pressure, in a weakly acidic aqueous sodium salt solution of from 10 to 30% concentration to raise the pH on the article to a value of greater than 1 and less than 7, and keeping the article in that solution at room temperature and under atmospheric pressure at least until the cellulose is completely regenerated.

2. The method of handling acid-moist articles freshly prepared from viscose, which articles comprise at least some partially regenerated cellulose and have a pH of less than 1 after withdrawal thereof from an acid setting bath, to effect complete regeneration of the cellulose by the acid while inhibiting acid degradation of the cellulose during and after such regeneration, and while the articles are held under acidic conditions comprising storing the article, at room temperature and under atmospheric pressure, in a weakly acidic aqueous sodium sulfate solution of from 10 to 30% concentration to raise the pH on the article to a value of greater than 1 and less than 7, and keeping the article in that solution at room temperature and under atmospheric pressure at least until the cellulose is completely regenerated.

3. The method of handling acid-moist articles freshly prepared from viscose, which articles

comprise at least some partially regenerated cellulose and have a pH of less than 1 after withdrawal thereof from an acid setting bath, to effect complete regeneration of the cellulose by the acid while inhibiting acid degradation of the cellulose during and after such regeneration and while the articles are held under acidic conditions, comprising storing the article, at room temperature and under atmospheric pressure, in a weakly acidic aqueous sodium salt solution of a concentration in the range of from 10 to 30% and such that the pH on the article is raised to and maintained at a value of from about 2 to 3.5, and keeping the article in that solution at room temperature and under atmospheric pressure at least until the cellulose is completely regenerated.

4. The method of handling acid-moist articles freshly prepared from viscose, which articles comprise at least some partially regenerated cellulose and have a pH of less than 1 after withdrawal thereof from an acid setting bath, to effect complete regeneration of the cellulose by the acid while inhibiting acid degradation of the cellulose during and after such regeneration, and while the articles are held under acidic conditions comprising storing the article, at room temperature and under atmospheric pressure, in a weakly acidic aqueous sodium sulfate solution of from 15 to 20% concentration to raise the pH on the article to a value of from about 2 to 3.5, and keeping the article in that solution at room temperature and under atmospheric pressure at least until the cellulose is completely regenerated.

5. The method of handling acid-moist filamentary material freshly prepared from viscose, which material comprises at least some partially regenerated cellulose and has a pH of less than about 1 after withdrawal from an acid setting bath, to effect complete regeneration of the cellulose by the acid while inhibiting acid degradation of the cellulose during and after such regeneration and while the material is held under acidic conditions which comprises collecting the filamentary material in the form of a wound package, storing the package, at room temperature and under atmospheric pressure, in a weakly acidic sodium salt solution of from 10 to 30% concentration to raise the pH on the material to a value of greater than 1 and less than 7, and keeping the package in that solution at room temperature and under atmospheric pressure at least until the cellulose is completely regenerated.

6. The method of handling acid-moist filamentary material freshly prepared from viscose, which material comprises at least some partially regenerated cellulose and has a pH of less than about 1 after withdrawal from an acid setting bath, to effect complete regeneration of the cellulose by the acid while inhibiting acid degradation of the cellulose during and after such regeneration and while the material is held under acidic conditions, which comprises collecting the filamentary material in the form of a wound package, storing the package, at room temperature and under atmospheric pressure, in a weakly acidic sodium sulfate solution of from 10 to 30% concentration to raise the pH on the material to a value of greater than 1 and less than 7, and keeping the package in that solution at room temperature and under atmospheric pressure at least until the cellulose is completely regenerated.

7. The method of handling acid-moist filamentary material freshly prepared from viscose,

which material comprises at least some partially regenerated cellulose and has a pH of less than about 1 after withdrawal from an acid setting bath, to effect complete regeneration of the cellulose by the acid while inhibiting acid degradation of the cellulose during and after such regeneration and while the material is held under acidic conditions, which comprises collecting the filamentary material in the form of a wound package, storing the package, at room temperature and under atmospheric pressure, in a weakly acidic sodium salt solution of a concentration in the range of from 10 to 30% and such that the pH on the material is raised to and maintained at a value of from about 2 to 3.5, and keeping the package in that solution at room temperature and under atmospheric pressure at least until the cellulose is completely regenerated.

8. The method of handling acid-moist filamentary material freshly prepared from viscose, which material comprises at least some partially regenerated cellulose and has a pH of less than about 1 after withdrawal from an acid setting bath, to effect complete regeneration of the cellulose by the acid while inhibiting acid degradation of the cellulose during and after such regeneration and while the material is held under acidic conditions, which comprises collecting the filamentary material in the form of a wound package, storing the package, at room temperature and under atmospheric pressure, in a weakly acidic sodium sulfate solution of from 15 to 20% concentration to raise the pH on the material to a value of from about 2 to 3.5, and keeping the package in that solution at room temperature and under atmospheric pressure at least until the cellulose is completely regenerated.

9. The method of handling acid-moist filamentary material freshly prepared from viscose, which material comprises at least some partially regenerated cellulose and has a pH of less than about 1, after withdrawal thereof from an acid setting bath, to effect complete regeneration of the cellulose while inhibiting acid degradation of the cellulose during and after such regeneration, and while the material is held under acidic conditions, comprising storing the material, at room temperature and under atmospheric pressure on a thread-advancing reel in a weakly acidic aqueous sodium salt solution of from 10 to 30% concentration to raise the pH on the material to a value of greater than 1 and less than 7, and keeping the material on the reel in that solution at room temperature and under atmospheric pressure at least until the cellulose is completely regenerated.

10. The method of handling acid-moist filamentary material freshly prepared from viscose, which material comprises at least some partially regenerated cellulose and has a pH of less than about 1, after withdrawal thereof from an acid setting bath, to effect complete regeneration of the cellulose while inhibiting acid degradation of the cellulose during and after such regeneration, and while the material is held under acidic conditions, comprising storing the material, at room temperature and under atmospheric pressure on a thread-advancing reel in a weakly acidic aqueous sodium sulfate solution of from 10 to 30% concentration to raise the pH on the material to a value of greater than 1 and less than 7, and keeping the material on the reel in that solution at room temperature and under atmospheric pressure at least until the cellulose is completely regenerated.

11. The method of handling acid-moist filamentary material freshly prepared from viscose, which material comprises at least some partially regenerated cellulose and has a pH of less than about 1, after withdrawal thereof from an acid setting bath, to effect complete regeneration of the cellulose while inhibiting acid degradation of the cellulose during and after such regeneration, and while the material is held under acidic conditions, comprising storing the material at 10 room temperature and under atmospheric pressure on a thread-advancing reel in a weakly acidic aqueous sodium sulfate solution of a concentration in the range of from 10 to 30% and such that the pH on the material is raised to and 15 maintained at a value of from about 2 to 3.5, and keeping the material on the reel in that solution at room temperature and under atmospheric pressure at least until the cellulose is completely regenerated.

12. The method of handling acid-moist filamentary material freshly prepared from viscose, which material comprises at least some partially regenerated cellulose and has a pH of less than about 1, after withdrawal thereof from an acid setting bath, to effect complete regeneration of the cellulose while inhibiting acid degradation of the cellulose during and after such regeneration, and while the material is held under acidic conditions, comprising storing the material at room 30

temperature and under atmospheric pressure on a thread-advancing reel in a weakly acidic aqueous sodium sulfate solution of from 15 to 20% concentration to raise the pH on the material to a value of from about 2 to 3.5, and keeping the material on the reel in that solution at room temperature and under atmospheric pressure at least until the cellulose is completely regenerated.

WAYNE A. SISSON.  
MAMERTO M. CRUZ, JR.

#### REFERENCES CITED

The following references are of record in the file of this patent:

#### UNITED STATES PATENTS

| Number    | Name           | Date          |
|-----------|----------------|---------------|
| 1,576,529 | Mendel         | Mar. 16, 1926 |
| 1,576,530 | Mendel         | Mar. 16, 1926 |
| 1,580,843 | Mendel         | Apr. 23, 1926 |
| 1,930,803 | Harrison       | Oct. 17, 1933 |
| 2,090,339 | Bitter         | Aug. 17, 1937 |
| 2,133,244 | Baumert et al. | Oct. 11, 1938 |
| 2,309,072 | Burkholder     | Jan. 19, 1943 |
| 2,327,516 | Fink et al.    | Aug. 24, 1943 |

#### FOREIGN PATENTS

| Number  | Country       | Date          |
|---------|---------------|---------------|
| 481,565 | Great Britain | Mar. 11, 1938 |
| 719,024 | Germany       | May 30, 1937  |